

## UNITED STATES PATENT OFFICE

THOMAS H. ROGERS, OF WHITING, INDIANA, ASSIGNOR TO STANDARD OIL COMPANY,  
OF WHITING, INDIANA, A CORPORATION OF INDIANA

## REFINED VISCOUS HYDROCARBON OIL

No Drawing.

Application filed August 19, 1926. Serial No. 130,351.

In the use of highly refined viscous hydrocarbon oils (from which substantially all asphaltic constituents have been removed, for example, by treatment with strong or 5 fuming sulphuric acid) for the lubrication of turbines and in similar uses, it has been found that they rapidly disolor, become increasingly acid and their tendency to emulsify increases. It has now been found that 10 these defects in the use of such oils may be to a substantial extent remedied by the addition to such oils of very small proportions (in general not more than 0.1%) of aromatic compounds in which a hydroxyl or amino 15 group is attached to the ring. Thus pyrogallol, diphenylamine, gallic acid, dibutylresorcinol, betanaphthol and hydroquinone have been successfully employed for this purpose. Thus, in the case of a fuming acid 20 treated white distillate oil of about 80 sec. Saybolt viscosity at 100° F. which, without the addition of such a substance, increased in acidity from 0.01 to 25 mgm. KOH equivalent per gram of oil in 100 hours and markedly decreased in demulsifiability, when oxygen 25 was passed therethrough at a temperature of 100° C., the same oil to which 0.04% pyrogallol had been added showed no increase in acidity and no decrease in demulsifiability. 30 Under like conditions. The addition of 0.04 to 0.1% diphenylamine, of 0.002% gallic acid and of 0.05% dibutylresorcinol, under similar circumstances, prevented any but relatively slight changes in acidity and demulsifiability. Thus, the same oil containing 35 0.002% gallic acid showed an increase in acidity in 161 hours to only 2.5 mgm. KOH equivalent per gram of oil.

The proportions of the aromatic compounds added may be varied considerably. In general 0.1% or less is sufficient to produce a marked result.

The oils prepared in accordance with the present invention have the property of retaining their resistivity to a high degree on aging.

I claim:

1. The method of preventing acid formation and increase of emulsifiability in use of 50 highly refined viscous hydrocarbon oils

which comprises adding thereto a small proportion of an aromatic compound having a substituting group attached to the ring, said substituting group being of the class consisting of the hydroxyl and amino radicals.

2. The method of preventing acid formation and increase of emulsifiability in use of 55 highly refined viscous hydrocarbon oils which comprises adding thereto up to 0.1% of an amino-aromatic compound.

3. The method of preventing acid formation and increase of emulsifiability in use 60 of highly refined viscous hydrocarbon oils, which comprises adding thereto a small quantity of an amino compound having a 65 plurality of aromatic rings attached to the nitrogen atom.

4. The method of preventing acid formation and increase of emulsifiability in use of 70 highly refined viscous hydrocarbon oils which comprises adding thereto 0.04 to 0.1% of diphenylamine.

5. A highly refined white viscous hydrocarbon oil free from asphaltic constituents 75 and containing a small proportion of an aromatic compound having a substituting group attached to the ring, said substituting group being of the class consisting of the hydroxyl and amino radicals.

6. A highly refined white viscous hydrocarbon oil free from asphaltic constituents 80 and containing a small proportion of an amino-aromatic compound.

7. A highly refined white viscous hydrocarbon oil free from asphaltic constituents 85 and containing a small quantity of an amino compound having a plurality of aromatic rings attached to the nitrogen atom.

8. A highly refined white viscous hydrocarbon oil free from asphaltic constituents 90 and containing 0.04 to 1% of diphenylamine.

THOMAS H. ROGERS.